

April 30, 1929.

E. A. CHASE

1,711,043

STONE ORNAMENTATION AND PROCESS OF PRODUCING THE SAME

Filed Oct. 19, 1926

2 Sheets-Sheet 1



Fig. 2.



Fig. 3.

Tridentor  
E. A. Chase  
By Attorneys

Southington, Fay & Hawley

April 30, 1929.

E. A. CHASE

1,711,043

STONE ORNAMENTATION AND PROCESS OF PRODUCING THE SAME

Filed Oct. 19, 1926

2 Sheets-Sheet 2



Fig. 5.



Fig. 7.



Fig. 8.



Fig. 9.



Fig. 10.



Fig. 11.

Attorney  
Troy A. Chase  
By Attorneys

Southgate Fay & Hawley

## UNITED STATES PATENT OFFICE.

ELROY A. CHASE, OF NORTHFIELD, VERMONT.

## STONE ORNAMENTATION AND PROCESS OF PRODUCING THE SAME.

Application filed October 19, 1926. Serial No. 142,729.

This invention relates to a new form of stone ornamentation and to an improved process for producing such improved ornamentation.

5 It is customary to produce ornamental surface effects on granite and other similar stone by sinking the background with a sand blast, leaving the ornamental design on the original prepared surface of the stone. This 10 simple process is not entirely satisfactory, as the background thus produced has a smooth unbroken surface and lacks character and contrast.

A considerable improvement has been 15 heretofore achieved by providing a wire screen in the path of the sand blast when cutting the background, whereby a conventional design appears as slightly raised lines or ribs on the surface of the background. 20 Such a background, while affording more contrast, is limited in its application, as only a very few designs can be commercially produced by this method and these fixed designs are not always well adapted to the 25 requirements of a particular surface design.

It is the general object of my invention to provide stone ornamentation having a distinctive background which may be easily and economically produced, which will be 30 more flexible in its application than the screen background previously used, and which may be easily adapted or modified to suit specific surface design requirements.

My invention further relates to an improved method by which my improved background may be easily and economically produced.

A preferred disclosure of my invention is shown in the drawings, together with certain additional figures showing the adaptation of my invention to several different designs.

Referring to the drawings:

Fig. 1 is a plan view of a portion of a block of granite or similar stone, showing the first step in the production of my novel ornamentation;

Fig. 2 is a sectional elevation, taken along the line 2—2 in Fig. 1;

50 Fig. 3 is a view similar to Fig. 2 but showing the result after the sand blast has been once applied thereto;

Fig. 4 is a partial plan view illustrating the next step in the process;

55 Fig. 5 is a sectional elevation, taken along

the line 5—5 of Fig. 4 but showing the result attained by a second application of the sand blast;

Fig. 6 is a partial plan view of a finished ornamentation; and

Figs. 7 to 11 inclusive are detailed plan views illustrating different background designs which may be produced by my new method.

Referring particularly to Figs. 1 to 6, I will now describe my improved ornamentation and the method by which it is preferably produced. A block 20 of granite or other stone is first provided with a smooth or finished surface and is then coated with a layer 21 of a special gelatinous or glue-like substance, adapted to resist the sand blast and to protect the portions of the stone covered thereby.

The desired ornamental design 22 is formed in the coating 21 by removing portions of the coating, thus outlining the design in the gelatinous coating. Instead, however, of entirely removing the coating from the portions of the stone intended to form the background, as has been the previous practice, I merely remove narrow strips of the coating, thus producing a background formed of parallel bars 23 separated by relatively narrow slots or grooves in the coating.

Having thus prepared the surface as indicated in Figs. 1 and 2, I direct the sand blast against the surface in the usual manner, cutting away all unprotected portions of the stone to an intermediate depth, as indicated in Fig. 3 and forming lines or grooves 24. The lines 24 thus produced in the stone have sharp edges and are very clearly defined.

I then remove the gelatinous coating from the bars 23 forming the background, but leave the coating over the design 22, as shown in Fig. 4. The sand blast is then again directed against the stone, sinking the previously formed grooves 24 to a greater depth, and at the same time cutting down the now exposed bars 23 at a rapid rate. After the second application of the sand blast, the stone has the appearance indicated in section in Fig. 5 and in plan view in Fig. 6. Fig. 6 also shows the coating removed from the design 22 and from the border portions 25, so that the finished effect is disclosed.

Comparison of Fig. 4 with Fig. 6 will show that the deepening of the background, after the coating 21 is removed from the bars 23, tends to destroy the sharp clean-cut outlines of the grooves 24, as the sand will follow to a greater or less extent the crystalline formation of the stone. In this way I break up the stiff symmetrical outline of the design as it appears in Fig. 4 and produce the much more pleasing effect shown in Fig. 6 in which the background, while provided with a markedly contrasting surface, is nevertheless more or less irregular and avoids the conventionality of the designs previously produced.

Having described the method by which my improved background is produced, it will be evident that the design of the background depends entirely upon the particular selection of the portions of the coating over the background to be removed, and that by varying the form of the openings in the coating, the effect of the finished background may be similarly varied.

In Figs. 7 to 11, I have illustrated different background effects, all of which may be produced by my improved method by simply varying the design which is cut into the coating over the background. In Fig. 7, the bars are indicated as extending obliquely and as being broken up into long and short portions. In Fig. 8, the remaining portions are approximately circular in outline. In Fig. 9, small square projections are provided. In Fig. 10, the slots separating the bars are wave-like instead of straight. In Fig. 11, a conventionalized fleur-de-lis appears on the background.

It will be understood that the possible variations in background which may be produced by this method are almost without limit. It will also be noted that the application of the background to a particular surface design may be varied in different parts of the design and that many novel and beautiful effects may thus be produced.

The term "sand blast" is used broadly to indicate a forceful delivery of sand or other granular cutting material by a stream of air, steam or gas.

Having thus described my invention and the advantages thereof I do not wish to be limited to the details herein disclosed otherwise than as set forth in the claims, but what I claim is:

1. The process of ornamenting granite and similar stone which consists in providing a sand-resisting, gelatinous coating for a surface of the stone, removing portions of said coating to outline a surface design and a background design, sand-blasting the stone to less than the desired finished depth of cut, removing the coating from additional portions of the background, and thereafter

sand-blasting the stone a second time to finished depth.

2. The process of ornamenting granite and similar stone which consists in providing a sand-resisting, gelatinous coating for a surface of the stone, removing portions of said coating to outline a surface design and a background design, sand-blasting the surface design to its entire depth while thus protected, and sand-blasting the background to partial depth while protected and thereafter to finished depth after removal of the protecting coating therefrom.

3. The process of providing a diversified background on a stone surface which consists in protecting the surface thereof with a gelatinous coating, cutting a background design therein, sand-blasting the stone to cut the background design to partial depth, removing additional portions of said coating, and again sand-blasting the background to finished depth.

4. The process of providing a diversified background on a stone surface which consists in protecting the surface thereof with a gelatinous coating, cutting a background design therein, sand-blasting the stone to cut the background design to partial depth, removing the remaining coating from said background design, and thereafter sand-blasting all portions of the background to greater depth.

5. The process of providing a diversified background on a granite surface which consists in cutting a predetermined design in the portion forming the background, and thereafter sand-blasting the background and the design cut therein to greater depth by directing a sand blast against all parts of the background.

6. An ornamentation for a granite block comprising a finished surface having a surface design sharply sand-blasted therein and having a sunken background with a predetermined background design sand-blasted therein but said background design having its outlines irregularly modified and substantially following the crystalline grain of the granite.

7. An ornamentation for a granite block comprising a finished surface having a surface design sharply sand blasted therein, and having a sunken background with a predetermined background design sand blasted therein, but said background design having its outlines irregularly modified and substantially following the crystalline grain of the granite, the surfaces of said background design being also irregularly modified and substantially following the crystalline grain of the granite.

In testimony whereof I have hereunto affixed my signature.

ELROY A. CHASE.